

# United States Patent Office

2,983,681

Patented May 9, 1961

1

2,983,681

## LUBRICATING COMPOSITIONS

Gifford W. Crosby, River Forest, and Allen F. Millikan, Crystal Lake, Ill., assignors to The Pure Oil Company, Chicago, Ill., a corporation of Ohio

No Drawing. Filed May 14, 1957, Ser. No. 658,940

10 Claims. (Cl. 252—46.4)

This invention relates to lubricating oil compositions containing small amounts of sulfurized isoprenoid compounds and small amounts of organic compounds containing phosphorus, arsenic or antimony, which compositions exhibit improved antiwear properties and oxidation stability. More particularly, the invention relates to the discovery that the combination of sulfurized isoprenoid compounds and organophosphorus, organoarsenic or organoantimony compounds in lubricating oils forms a superior antiwear composition as exemplified by its performance in the four-ball extreme pressure machine, wherein a synergistic effect has been found to take place between the compounds of the aforeslated general classification.

Organocompounds of group VB elements, that is, phosphorus, arsenic, antimony and bismuth, are best known for their inhibition of oxidation processes, although certain of these compounds are described as having some extreme pressure properties when used in lubricating oil compositions. Similarly, sulfurized isoprenoid compounds are known for their ability to impart oxidation stability and non-corrosive properties to lubricating compositions used in the presence of alloyed bearings. Sulfurized isoprenoid compounds have in some instances been used for their extreme pressure properties. However, it is also well-known that complex addends of the types aforementioned, which are effective for improvement in detergency, oxidation resistance or corrosion resistance of lubricating oils, are often prone to produce high wear-rates when used in the lubrication of steel sliding on steel. Known detergents, oxidation inhibitors, and corrosion-preventing addends are generally considered to be ineffective as extreme pressure agents under the severe conditions that are found in modern extreme pressure tests, such as the Shell four-ball test.

The present invention is predicated on the unexpected discovery that the combination of antioxidants and detergents consisting of sulfur-containing isoprenoid compounds and organocompounds of phosphorus, arsenic and antimony exerts a synergistic antiwear effect and produces low wear-rates as measured by the four ball test. The extraordinary effect of the specific combination of addends of this invention is emphasized by the fact that one of the addends, namely the organocompounds of group VB elements, produces far greater wear with the mineral lubricating oil than the oil alone produces. Furthermore, it will be demonstrated that the unusual antiwear properties of the combination of addends of this invention is not shared by certain members of the broad group of addends into which they fall, such as combinations of amines or bismuthines, representing the remaining members of group VB compounds, with sulfurized isoprenoids.

Accordingly, a primary object of this invention is to provide an extreme pressure lubricating composition containing the combination of sulfurized isoprenoid compounds and organocompounds of elements of group VB of the periodic table (Welch Manufacturing Company,

2

revised edition, 1953), excluding bismuth and nitrogen.

The isoprenoid compounds which are employed to produce the sulfurized derivatives used as a part of the composition of this invention include the alicyclic, monocyclic, and dicyclic terpene hydrocarbons, and are well-known in the art. The terpenes have the general formula  $C_{10}H_{16}$  and many are diolefinic derivatives of cyclohexane. The more complex alicyclic terpenes are the sesquiterpenes,  $C_{15}H_{24}$ , and the polyterpenes ( $C_5H_8$ ) $n$ . Among the open-chain terpene derivatives are 2,6-dimethyloctatriene, geraniol, linalool, citronellol, citroellal and rhodinal. Among the monocyclic terpenes which are considered to be derivatives of p-menthane, or 1-methyl-4-isopropylcyclohexane, are  $\alpha$ -terpinene, gamma-terpinene,  $\alpha$ -phelandrene,  $\beta$ -phelandrene, terpinolene, limonene and menthol,  $\beta$ -terpinene and pseudolimonene. The most important monocyclic terpenes are limonene,  $\alpha$ -terpinene and  $\alpha$ -phelandrene. Para-menthane may be derived from menthol by reduction, menthol being associated with terpenes in essential oils. Other oxidation derivatives of p-menthane, also associated with terpenes in essential oils, are carvomenthol, pulegone,  $\alpha$ -terpineol, menthane and carvone.

d-Limonene is found in all citrus oils. 1-limonene occurs in pine needles and fir cones and oil of peppermint. The racemic modification, dipentene, is found in many essential oils. Dipentene is found in turpentine and obtained by the distillation of pine wood. Dipentene may be regarded a dimer of isoprene and may be produced therefrom by polymerization.  $\alpha$ -Terpineol can be formed from the dehydration of terpin hydrate which may be produced from dipentene or geraniol.

Among the dicyclic terpenes which are considered to be cyclohexane with a bridge of one or more carbon atoms, the most important members are carene, pinene, and camphane. These dicyclic isoprenoids may be considered to be derivatives of p-menthane by having the isopropyl group close a bridging ring across the cyclohexane ring.  $\alpha$ - and  $\beta$ -Pinene are obtained, the former in a proportion of 90%, by distillation of the yellow pine resin exudate from pine trees. Turpentine oils contain two homologues of benzene in the form of m-cymene and p-cymene. Terpinolene, a monocyclic diene, is prepared synthetically from terpineol by dehydration with oxalic acid.

Fenchone is another bicyclic terpene derivative under the camphane group and is isomeric with camphor. The treatment of  $\alpha$ -pinene with dry hydrogen iodide produces bornyl iodide which on reduction yields camphane.

The isoprenoid compounds found in naval stores products may be used, such as the constituents of  $\alpha$ -pinene, gum and wood turpentine, and the constituents of dipentene 122 or pine oils. Specifically, these materials range from cyclofenchene boiling at about 143° C. to  $\alpha$ -terpineol boiling at 237° C., including such well-known isoprenoids as  $\alpha$ -pinene, camphene,  $\beta$ -pinene,  $\alpha$ -terpinene, dipentene, p-cymene, gamma-terpinene, 2,4(8)-para-menthadiene and terpinolene.

Typical commercial proprietary terpene products by the Hercules Powder Company include wood turpentine, Dipentene 122, Hercosol 80, Solvenols 1 and 2, Yarmor pine oil, B-3 reagent and terpineol 318. Dipentene 122, for example, is a trade name for a mixture of mono- and dicyclic terpenes, including dipentene,  $\alpha$ -terpinene, terpinolene,  $\alpha$ -pinene,  $\beta$ -pinene, and 2,4(8)-para-menthadiene with considerable amounts of p-cymene and p-menthane.

The sulfurized products of the aforementioned isoprenoid compounds may be prepared by any of the many methods disclosed in the prior art. The methods de-

scribed in the following United States Patents may be used:

- 1,844,400—Kobbe  
2,417,305—Knowles  
2,443,823—Holt  
2,689,846—Beegle

In general, the sulfurization of the isoprenoid is carried out by adding an amount of sulfur which is stoichiometrically in excess of the amount required to react with the double bonds present in the isoprenoid, and heating the mixture in a kettle or stainless steel autoclave at temperatures ranging from 250° F. to 400° F. for a time sufficient to complete the reaction. The isoprenoid compound used should have at least one unsaturation in the molecule. In general, it is preferred to use ordinary flowers of sulfur during the sulfurization step in proportions of about 20 to 35 parts by weight, especially 25 to 30 parts of sulfur, for each 100 parts of reaction mixture, or about 25 to 54%, based on the weight of isoprenoid compound. The ingredients may be combined by heating the isoprenoid compound and adding the sulfur thereto; or, the sulfur may first be melted and the terpene added gradually thereto; or, the ingredients may be combined without prior heating and thereafter heated together to a temperature above the melting point of the sulfur. This is followed by further heating to about 300 to 400° F. Non-limiting examples follow:

#### EXAMPLE I

Three hundred grams of terpinolene and 90 grams of sulfur are mixed and placed in a 1000 cc. stainless steel autoclave. Heat is applied and the mixture is maintained at about 340° F. for about 30 minutes. The temperature is raised to about 360° F. for another 30 minutes with agitation. A pressure of about 50 p.s.i.g. develops. The autoclave is then cooled and the reaction mixture is subjected to vacuum steam-stripping to 300° F. at about 15 mm. Hg. The product may be used as such, or purified by dilution with an equal volume of benzene and refluxed with agitation for four hours at 185–190° F. in the presence of a solution consisting of about 600 grams of water, 300 grams of sodium sulfide ( $\text{Na}_2\text{S} \cdot 9\text{H}_2\text{O}$ ), and 100 grams of sodium hydroxide. The mixture is then allowed to cool, 500 cc. of pentane are added and the mixture is shaken. A bottom layer of a dark orange-red liquid is drawn off and the upper layer is washed several times with water. This top layer is filtered and the benzene and pentane is removed by evaporation on a steam bath. The product, sulfurized terpinolene, is a yellow-brown liquid containing about 29 to 30% sulfur.

#### EXAMPLE II

Two hundred grams of steam-distilled pine oil, containing as its main constituent alpha-terpineol (B.P. 422°–424° F.), is heated at 220° F. with 50 grams of sulfur. As the temperature rises, the sulfur melts and dissolves in the pine oil. When the temperature reaches about 350° F., ebullition takes place and an exothermic reaction begins which brings the temperature to about 375° F. After heating for 4–5 hours at 375–400° F., a homogeneous mass is obtained and purification is carried out as in Example I.

#### EXAMPLE III

By heating 600 grams of terpinolene to 330° F. in a three-neck flask equipped with a mercury-seal stirrer and two reflux condensers, adding gradually 180 grams of sulfur through one of the condensers at a rate to maintain the temperature at 350° F., heating to about 350° F. for 2½ hours, cooling, filtering, and vacuum steam-stripping to 300° F. and purifying in accordance with Example I, a product containing about 29% sulfur, a yellowish-brown oil, is obtained.

The organocompounds of phosphorus, arsenic and antimony to be used in accordance with this invention may

have organic radicals of the aliphatic, carbocyclic, including alicyclic and aromatic, and heterocyclic series having a total of from 3 to 30 carbon atoms. Thus, the phosphines, arsines and stibines include compounds which contain the specific groups of trimethyl, dimethylethyl, methylethylpropyl, methylethylcetyl, dibutylcetyl, triethyl, tripropyl, trisopropyl, tributyl, triamyl, dimethylbutyl, tricetyl, methylidiphenyl, diethylbenzyl triphenyl, tritolyl, and tripyridyl. Other specific compounds include dibutylphenylphosphine, dilaurylphenylphosphine, and diwaxphenylphosphine. Particularly applicable to the invention are those organocompounds of phosphorus, arsenic and antimony in which the organo portion of the molecule contains only carbon and hydrogen.

In order to illustrate the invention, a number of lubricating compositions were prepared and subjected to tests on the shell four-ball EP machine in which a steel ball is rotated in contact with 3 stationary balls submerged in the test oil. This machine may be used to determine characteristic properties such as wear-rate under various conditions, load-carrying capacity, or ability to prevent seizure and welding under high loads. The test used to evaluate the oils of this invention was a wear test of 5 minutes duration, a rotational speed of 1800 r.p.m. for the top ball, and an applied load of 20 kg. Wear measurements are the average diameter in mm. of the scars produced by the rotating ball on the three stationary balls. A low-wear lubricant will produce a scar diameter only slightly greater than the diameter of elastic indentation of the balls, which in the case of the stated load and ball composition used is 0.24 mm. Table I shows some results obtained with the compositions of our invention containing triphenyl derivatives of group VB elements.

Table I

| Lubricant Composition, Wt. Percent |         |             |                    |                    | 4-Ball Wear Test     |                                                |
|------------------------------------|---------|-------------|--------------------|--------------------|----------------------|------------------------------------------------|
| Group V Organo-compound            | Element | Wt. Percent | Sulfurized terpene | Basic Ba-Sulfonate | 170 vis. Mineral Oil | Increase in av. scar dia. over Hertz dia., mm. |
|                                    |         |             |                    |                    |                      |                                                |
| 40                                 |         |             |                    |                    |                      |                                                |
| 45                                 | Sb.     | 1.1         | 0.7                | 5.3                | 98.2                 | 0.03                                           |
|                                    | Sb.     | 1.1         | 0.7                | 5.3                | 92.9                 | 0.03                                           |
|                                    | Sb.     | 1.1         | 0.7                | 5.3                | 98.9                 | 0.34                                           |
|                                    | As.     | 1.0         | 0.7                | 5.3                | 93.0                 | 0.03                                           |
|                                    | As.     | 1.0         | 0.7                | 5.3                | 99.0                 | 0.04                                           |
|                                    | P.      | 0.8         | 0.7                | 5.3                | 98.5                 | 0.02                                           |
|                                    | P.      | 0.8         | 0.7                | 5.3                | 99.2                 | 0.05                                           |
|                                    |         |             | 0.7                | 5.3                | 94.0                 | 0.12                                           |
|                                    |         |             | 0.7                | 5.3                | 99.3                 | 0.08                                           |
|                                    |         |             |                    |                    | 100.0                | 0.14                                           |
|                                    | N.      | 0.8         | 0.7                | 5.3                | 93.2                 | 0.09                                           |
|                                    | N.      | 0.8         | 0.7                | 5.3                | 99.2                 | 0.13                                           |
|                                    | Bi.     | 1.4         | 0.7                | 5.3                | 92.6                 | 0.20                                           |

It will be seen from Table I that antiwear properties are exhibited to a marked degree by oil blends containing the additive combination of sulfurized terpene and a phosphine arsine or stibine. The antiwear properties are also maintained in the presence of a commonly used motor oil detergent additive, basic barium petroleum sulfonate. In this table the average wear values were obtained from three or more individual runs for each lubricant. The individual additives do not necessarily show antiwear properties; in fact, triphenylstibine in mineral oil shows a higher wear rate than mineral oil alone. Examples of oil blends containing organocompounds of the other two elements of group VB, viz., nitrogen and bismuth, are included to compare the inferior wear protection afforded by combinations of additives containing these two elements with the sulfurized terpene.

Components of the above lubricant compositions may be further identified as follows. The organocompounds of group VB elements with which this invention is con-

cerned were all triphenyl derivatives and equivalent molar concentrations were used. The sulfurized terpene was a commercial product containing 29.4 wt. percent sulfur and having a specific gravity of 1.164. The sulfonate was a commercial basic barium petroleum sulfonate containing 15.9 wt. percent sulfated ash, and having a total base number of 30. The mineral oil in the above blends was a Mid-Continent solvent-refined neutral oil with a viscosity of 170 SUS at 100° F.

Although the lubricating oil compositions of this invention are illustrated by compositions containing a major proportion of a neutral oil, a minor proportion of a compound selected from the group consisting of triphenylstibine, -arsine, and -phosphine, used at a concentration of 0.8 to 1.1 wt. percent, and a minor proportion of a product characterized as a sulfurized terpene, used at a concentration of 0.7 wt. percent, it is to be understood that the invention encompasses alkyl, aryl, alkaryl, arylalkyl, carbocyclic, including alicyclic and aromatic and heterocyclic phosphines, stibines and arsines, in which the organic radicals are the same or different. It is apparent also that other lubricating oil fractions may be used and that the proportions of the different constituents may vary within the broad limits disclosed. Other additives, such as detergents and pour depressants normally used in modern motor oil formulations, can also be incorporated while maintaining the advantages of the preferred combination of sulfurized terpene and triphenylstibine, arsine or phosphine, or other antiwear additive combinations as set forth herein.

What is claimed is:

1. A lubricating composition comprising a major portion of a mineral lubricating oil, about 0.2 to 5.0 weight percent of a sulfurized terpene compound selected from the group consisting of sulfurized pine oil, sulfurized terpinolene, sulfurized dipentene and sulfurized pinene, and about 0.2 to 5.0 weight percent of an organocompound selected from the group of triphenylphosphine and triphenylstibine said sulfurized terpene compounds and said organo-compound being essentially the only antiwear constituents present in said composition.

2. A lubricating composition comprising a major por-

tion of a mineral lubricating oil and about 0.7 weight percent of a sulfurized terpene compound selected from the group consisting of sulfurized pine oil, sulfurized terpinolene, sulfurized dipentene and sulfurized pinene and about 0.8 to 1.1 weight percent of an organo-compound selected from the group consisting of triphenylphosphine and triphenylstibine said sulfurized terpene compound and said organo-compound being essentially the only antiwear constituents present in said composition.

3. The lubricating composition of claim 2 in which the sulfurized terpene compound is sulfurized pinene.

4. The lubricating composition of claim 2 in which the sulfurized terpene compound is sulfurized pine oil.

5. The lubricating composition of claim 2 in which the sulfurized terpene compound is sulfurized terpinolene.

6. The lubricating composition of claim 2 in which the sulfurized terpene compound is sulfurized dipentene.

7. The lubricating composition of claim 2 in which the organocompound is triphenylphosphine.

8. The lubricating composition of claim 2 in which the organocompound is triphenylstibine.

9. An extreme pressure lubricant comprising a major portion of a mineral lubricating oil, about 0.7 weight percent of sulfurized terpene and about 1.1 weight percent of triphenylstibine said sulfurized terpene and said triphenylstibine being essentially the only antiwear constituents present in said lubricant.

10. An extreme pressure lubricant comprising a major portion of a mineral lubricating oil, about 0.7 weight percent of sulfurized terpene and about 0.8 weight percent of triphenylphosphine said sulfurized terpene and said triphenylphosphine being essentially the only antiwear constituents present in said lubricant.

#### References Cited in the file of this patent

#### UNITED STATES PATENTS

|           |         |               |
|-----------|---------|---------------|
| 2,149,271 | Butz    | Mar. 7, 1939  |
| 2,334,566 | Lincoln | Nov. 16, 1943 |
| 2,443,823 | Holt    | June 22, 1948 |
| 2,643,248 | Brennan | June 23, 1953 |